

## UNITED STATES PATENT OFFICE

2,085,544

## ACID RESISTANT COPPER ALLOYS

William B. Price, Waterbury, Conn., assignor to  
Scovill Manufacturing Company, Waterbury,  
Conn., a corporation of Connecticut

No Drawing. Application October 13, 1936,  
Serial No. 105,442

5 Claims. (Cl. 75—154)

This invention relates to acid resistant copper alloys; and it comprises as a quaternary alloy of copper a physically homogeneous solid solution of small grain size and of good tensile strength without brittleness combined with easy workability and containing 2 to 3 per cent each of nickel, aluminum and tin with 94 to 91 per cent copper; all as more fully hereinafter set forth and as claimed.

10 Copper metal is not attacked by acids or alkalies in the absence of oxygen. It is, however, oxidized by moist air and in the presence of oxygen the metal is corroded and dissolved by most acids. Pure copper is so soft that it is difficult 15 to machine. Its tensile strength is comparatively low. For use as sheets, bars, wire, tubes, rivets, rods, bolts, nuts and the like, copper is mostly alloyed with other metals. In these alloys the inherent properties of copper metal are drastically changed. It is an object of the present invention, by alloying the copper with other metals, to increase the strength and hardness and lessen the ductility and malleability of copper metal to the proper extent to make it practically workable by modern commercial machine methods 20 and to increase its resistance to acid oxidation attack without interfering with the workability of the metal and without making it brittle.

I have found that when copper is alloyed with about 6 to 9 per cent of the three alloying metals, nickel, aluminum and tin together, and when these three alloying metals are present in substantially equal proportions, these objects are attained: a copper alloy is produced of excellent 30 mechanical properties, high resistance to corrosion and of outstanding excellence for many purposes such as heat exchanger tubing. The alloy of copper with small amounts of nickel, aluminum and tin is greatly superior, in the above identified respects, to those composed of copper, nickel and aluminum, or of copper, nickel and tin. For example, I have found that an acid 35 resistant, workable alloy of 90 to 94 per cent copper 3 to 5 per cent aluminum and 3 to 5 per cent nickel, is greatly improved by replacing substantially equal fractions of both the aluminum and the nickel with tin. The total percentage of the alloying components is not substantially changed but the replacement by tin of 40 about one-third of the aluminum and one-third of the nickel, adds to the acid oxidation resistance of the metal alloy, improves its workability by modern machine methods and makes a generally improved metal for use in the form of 45 sheets, bars, wire, tubes, rivets, rods, bolts, nuts, etc. In particular, the quaternary alloy of cop-

per, nickel, aluminum and tin in the stated proportions gives an improved metal for use in making condenser tubes. As stated, the quaternary alloy is more resistant to acids, alkalies and oxidation-corrosion, is stronger, less brittle and more readily workable than the ternary alloys of copper with nickel and aluminum.

This quaternary alloy of copper with small amounts of nickel, aluminum and tin appears to be a true solid solution of the four metals. The 10 physical structure of the metal after heat treatment of the cast metal by usual methods is made up of small size grains, usually not larger than 0.012 mm., and appears to be completely homogeneous.

I find that the total combined percentage of the three alloying metals added to the copper should be kept within the range of 6 to 9 per cent of the alloy, the copper ranging between 94 and 91 per cent. With substantially more than 9 20 per cent of Ni, Al and Sn combined and less than 91 per cent copper, the metal becomes brittle and unworkable and with more than 94 per cent copper and less than 6 per cent of Ni, Al and Sn the metal is too soft and low in tensile strength. 25 However, some latitude is allowable in the respective proportions of the three alloying additions. For example, the aluminum may run slightly below 2 per cent of the alloy and the nickel and tin proportionately above 2 per cent 30 each. Small amounts of other metals, as for example iron and manganese, existing as impurities do not alter the properties of the alloy, so long as the relative proportions of the four metals in the quaternary alloy are not materially affected.

In making a copper alloy resistant to acid oxidation attack and also strong and workable, it has been known that aluminum and nickel together in small ratios to the copper are effective. 40 Copper of course has been alloyed with various large and small proportions of nickel and in these copper-nickel alloys small percentages of tin, running from 1 per cent to around 5 per cent, have improved both the workability and also the 45 resistance to oxidation and acid corrosion.

The quaternary alloy is made by melting the constituent metals together in a clay graphite crucible heated in an electric furnace. Advantageously pure nickel shot may be placed in the bottom of the crucible and an alloy of 95 per cent copper with 5 per cent aluminum melted down over the nickel shot with sufficient pure copper added to give the required ratio. The mixture in the crucible is held under a charcoal 50 55

cover to complete the fusion and the tin is added with thorough admixture before skimming the melt and pouring into oiled warm cast iron moulds. It is usually advantageous to deoxidize the melt just before pouring by a small addition of magnesium.

The following examples A, B and C are given of the quaternary copper base alloys of the present invention.

10 Alloy A analyzes as 93.85 per cent copper, 2.43 per cent tin, 2.31 nickel and 1.64 per cent aluminum. The tensile strength is good, the metal exhibits an exceptionally fine-grained structure and has a high acid resistance. Metal of 0.035 15 gauge, and of 8 degrees hardness has a tensile strength of 102,000 pounds per square inch with 2 per cent elongation. The tensile strength drops on annealing and quenching but can be reinstated by reduction in rolling.

20 Tabulated, the properties of this alloy are:

|    | Description                                | Gauge inch | Lbs/sq. in. tensile strength | Percent elong. 2" | Rockwell No. (1/16" 100 kg.) | Remarks                                      |
|----|--------------------------------------------|------------|------------------------------|-------------------|------------------------------|----------------------------------------------|
| 25 | No. 8 hard                                 | .035       | 102,000                      | 2.0               | B 95                         |                                              |
|    | Annealed at 500° C.                        | .035       | 70,000                       | 23.0              | B 77                         |                                              |
|    | Annealed at 650° C.                        | .035       | 58,000                       | 32.0              | B 61                         |                                              |
| 30 | Quenched from 900° C.                      | .035       | 46,000                       | 53.0              | B 33                         |                                              |
|    | Quenched aged 2 hrs. @ 650° C.             | .035       | 47,500                       | 42.0              | B 43                         |                                              |
|    | Quenched rolled 50%.                       | .047       | 90,000                       | 4.0               | B 92                         |                                              |
| 35 | Quenched rolled 50%, aged 2 hrs. @ 650° C. | .047       | 56,000                       | 38.0              | B 57                         | Completely recrystallized, gr. size .012 mm. |
|    | Quenched rolled 75%.                       | .022       | 107,000                      | 2.0               | B 97                         |                                              |
|    | Quenched rolled 75%, aged 2 hrs. @ 650° C. | .023       | 55,000                       | 35.0              | B 64                         | Completely recrystallized, gr. size .012 mm. |

40 Alloy B, a second alloy, analyzes 92.57 per cent copper, 2.09 per cent tin, 2.32 per cent nickel and 2.51 per cent aluminum with 0.57 per cent manganese. The tin is a little less and the aluminum a little higher, but the alloy has properties quite similar to those of alloy A. There is but little tendency for these alloys to become hardened by the aging heat treatments.

45 The third alloy C analyzes 90.89 per cent copper, 3.16 per cent tin, 2.23 per cent nickel and 3.23 per cent aluminum. In this alloy the cop-

per is somewhat less and there are variations in amount of the three metals. The alloy shows the following characteristics:

| Description                              | Gauge inch | Lbs/sq. in. tensile strength | Percent elong. 2" | Rockwell No. (1/16" 100 kg.) | 5  |
|------------------------------------------|------------|------------------------------|-------------------|------------------------------|----|
| Quenched from 650° C.                    | .025       | 68,200                       | 40.0              | B 67                         |    |
| Quenched aged 2 hrs @ 375° C.            |            | 70,800                       | 31.0              | B 71                         | 10 |
| Quenched aged 2 hrs @ 425° C.            |            | 73,200                       | 26.0              | B 74                         |    |
| Quenched rolled 50%                      |            | 119,700                      | 2.0               | B 99                         |    |
| Quenched rolled 50% aged 2 hrs @ 375° C. |            | 114,700                      | 4.0               | B 100                        |    |
| 400° C.                                  |            | 110,900                      | 4.0               | B 99                         |    |
| 425° C.                                  |            | 99,400                       | 14.0              | B 95                         |    |
| Quenched rolled 75%                      |            | 125,600                      | 1.0               | B 101                        |    |
| Quenched rolled 75% aged 2 hrs @ 375° C. |            | 119,500                      | 3.0               | B 101                        |    |
| 400° C.                                  |            | 106,000                      | 11.0              | B 98                         |    |
| 425° C.                                  |            | 92,200                       | 16.0              | B 93                         |    |

20

#### What I claim is:—

1. An acid and oxidation resistant physically homogeneous and easily workable copper alloy consisting substantially of copper, nickel, aluminum and tin in the proportions of

25

|          |          |          |
|----------|----------|----------|
| Copper   | 94 to 91 | Per cent |
| Nickel   | 2 to 3   |          |
| Aluminum | 2 to 3   |          |
| Tin      | 2 to 3   | 30       |

2. A quaternary copper alloy composed of 94 to 91 per cent copper alloyed with 6 to 9 per cent of nickel, aluminum and tin in substantially equal proportions of the three alloying metals.

35

3. A copper-nickel-aluminum-tin alloy consisting of about 9 per cent of nickel, aluminum and tin combined and about 91 per cent copper and containing approximately equal proportions of the nickel aluminum and tin.

40

4. An alloy of about 91 to 94 per cent copper with less than about 9 per cent and more than about 6 per cent nickel and aluminum in approximately equal proportions, characterized by having approximately one-third of the nickel and one-third of the aluminum replaced by tin.

45

5. A copper-nickel-aluminum-tin alloy composed of about 94 per cent copper alloyed with a total of about 6 per cent of nickel, aluminum and tin in approximately equal proportions.

50

WILLIAM B. PRICE.